

84 -M

Patented Mar. 10, 1931

1,795,639

## UNITED STATES PATENT OFFICE

JACK CHAMBERS CHASTON AND JOHN PERCY JOHNS, OF ALDWYCH, LONDON, ENGLAND,  
ASSIGNORS TO WESTERN ELECTRIC COMPANY, INCORPORATED, OF NEW YORK, N. Y.,  
A CORPORATION OF NEW YORK

### MAGNETIC STRUCTURE

No Drawing. Application filed September 21, 1928, Serial No. 394,381, and in Great Britain October 4, 1928.

This invention relates to the manufacture of magnetic structures such as cores for loading coils and the like, of the type in which finely divided magnetic particles, mixed with an insulating material, are compressed into a suitable form.

In this manufacture it is necessary to use considerable pressure in order to obtain a core of high permeability, and if the magnetic material is of such character that its permeability is sensitive to strain, very many problems arise as to the treatment, components and conditions for producing a most satisfactory structure. This is most noticeable where

15 the magnetic material is a nickel iron alloy, for although this alloy is capable of having developed in it an extremely high permeability this permeability is very considerably reduced by mechanical strain. Thus, though 20 a high degree of compression must be reached, the magnetic particles in the finished core should during and after the subsequent heat treatment be as far as possible free from strain.

25 An object of the present invention is to change a physical characteristic of the insulating material between the compression stage and the subsequent heat treatment.

This may be effected by subjecting the core 30 after compression and prior to the final annealing treatment, to a fluid, for a length of time sufficient for the desired physical characteristics to be obtained.

35 In the preferred form of the invention the fluid is one which being partly absorbed by the insulation causes it to swell and during a subsequent heat treatment is liberated, at least partially. If the insulating material comprises chromic acid and/or sodium silicate or such other hygroscopic substance, the fluid may be water, water vapour or a humid atmosphere. In this case it may be desirable 40 to dry the core immediately prior to the annealing treatment. Cores made according to 45 the invention have been found to give very low hysteresis losses and the invention also enables a greater control to be exercised over the permeability of the finished core.

50 It is believed that the improvements are due to the reduction of strain in the magnetic

particles of the heat treated core. A consideration of the action of pressing shows that during this operation the particles are permanently deformed and moulded so as to fit closely together and interlock. Unless permanent deformation takes place the particles will not be able to fit together sufficiently closely to give the desired values of permeability to the finished cores. The use of lower pressures would produce less strain, but the particles would not be keyed together satisfactorily, spaces would remain between the particles, and the permeability would be low. It seemed that if the particles could be caused to move slightly apart after the compression 55 and then given more freedom to move, the setting up of strains would be reduced. Thus by causing the insulation to perform this function, an improved core was produced.

The invention may be carried out in the 60 following manner:—

A magnetic dust is prepared from an alloy containing about 80% nickel and the remainder iron. It is desirable to anneal the particles at this stage. The annealed particles 65 are then mixed with chromic acid, sodium silicate and talc in the same manner and proportions as described in the U. S. patent to J. W. Andrews et al., No. 1,669,643, issued May 15, 1928. The mixture is then compressed 70 into core form preferably with a pressure of approximately 200,000 pounds per square inch as in the method disclosed in the aforementioned patent. The core is allowed to hang freely in an atmosphere of definite humidity 75 for a given length of time. The degree of humidity of the air in the conditioning chamber, the temperature of the air, and the time of conditioning may be varied over wide limits. In general, the effect of conditioning becomes more marked as the humidity is raised, but there seems to be little advantage 80 in employing a higher humidity than that of saturated air at room temperature.

85 Good results have been obtained by conditioning the core rings for 18 hours in a closed vessel in which the air is maintained saturated with water vapor at room temperature. After this treatment the cores are preferably 90 subjected to a final annealing heat treatment. 95

103.8  
40  
45  
50  
55  
60  
65  
70  
75  
80  
85  
90  
95  
100

similar to that disclosed in the aforesaid patent, after which they are ready for service. Measurements made on a typical batch of core rings conditioned in this manner showed them to have a core loss of 68.4 ohms per henry when tested at a frequency of 3000 cycles per second. Similar cores having the same permeability, but which were not conditioned, were found to have a core loss of 89.1 ohms per henry when tested under similar conditions.

The operation of conditioning thus resulted in a reduction of the core loss amounting to 23.3%.

Instead of conditioning in moist air, the cores may be placed in water, thus going to the limit of humidity. The effect to this treatment as regards improvements in magnetic properties is substantially the same as if the rings were kept in saturated air at room temperature, but there is a tendency for the mechanical strength of the cores to be impaired when the cores are immersed in water, and, therefore, the treatment with humid air is preferable. If the water treatment is used care must be taken to limit the time of exposure to the water or the cores may fall to pieces.

Although the invention has been described by way of example with particular reference to specific insulating and conditioning mediums, it will be clear that other insulating materials and conditioning fluids may be used and in fact that any insulating material may be used, the physical characteristics of which may be changed by conditioning in any suitable fluid between the compression stage and the subsequent heat treatment.

Also, though the invention has been described with particular reference to the manufacture of cores, it will be clear that it may be employed in the manufacture of structures of any other form which are made by compressing insulated finely divided magnetic particles.

What is claimed is:

1. A method of producing a magnetic structure or core which comprises insulating particles of magnetic material, compressing the insulated particles to a suitable form, subjecting the insulated, compressed particles to a fluid substance for a sufficient length of time to appreciably change the physical characteristics of the insulating material, and heat treating the resulting product.

2. A method of producing a magnetic structure comprising magnetic particles insulated from each other, wherein the core after being compressed, and previous to an annealing heat treatment, is subjected to a fluid until the physical properties of the insulating material are appreciably modified whereby the magnetic characteristics produced in the final heat treatment may be fully developed.

3. A method of producing a magnetic structure which comprises insulating magnetic particles, compressing the insulated particles into a homogeneous body, subjecting said body to a fluid for a sufficient length of time to cause the insulation therein to swell appreciably, and heat treating the resulting product.

4. The method of claim 1 in which said compressed insulated particles are subjected to said fluid for a time sufficient to enable an appreciable portion of said fluid to be absorbed by the insulation, at least a portion of which fluid is liberated during the subsequent annealing heat treatment.

5. The method of claim 1 and in which said insulating material comprises a hygroscopic substance, and said fluid includes water.

6. The method of claim 1 and in which said magnetic particles are insulated with an insulating material including chromic acid and sodium silicate.

7. The method of claim 1 and in which said magnetic material comprises an alloy including nickel and iron.

8. The method of claim 1 and in which said fluid substance is in vapor form.

9. The method of claim 1 in which the fluid substance to which the insulated compressed particles are subjected comprises air saturated with water vapor.

In witness whereof, we hereunto subscribe our names this twentieth day of August, 1929.

JACK CHAMBERS CHASTON. 100  
JOHN PERCY JOHNS.

105

110

115

120

125

130